# EUROPEAN PATENT APPLICATION

(11) **EP 4 694 576 A1**
(43) Date of publication of application: **11.02.2026**
(21) Application number: 24780535.1
(22) Date of filing: 27.03.2024
(51) Int. Cl.: H05B 3/20

(54) **LAYERED BODY**

(30) Priority: 29.03.2023 JP 2023053161
(71) Applicant: LINTEC CORPORATION, Itabashi-ku Tokyo 173-0001 (JP)
(72) Inventor: OSHIMA, Takuya, Tokyo 173-0001 (JP); ITO, Masaharu, Tokyo 173-0001 (JP)
(74) Representative: Gille Hrabal Partnerschaftsgesellschaft mbB Patentanwälte
(86) International application number: PCT/JP2024/012440
(87) International publication number: WO 2024/204434

(57) **Abstract**

A laminate (100) includes: a first base material (1); a second base material (2) having a higher linear coefficient of thermal expansion than the first base material (1); and a wiring sheet (10) held between the first base material (1) and the second base material (2), in which the wiring sheet (10) includes a wiring body (3) including a plurality of electrically conductive linear bodies (31) arranged with a spacing, a first resin layer (4) directly or indirectly supporting the wiring body (3), and a pair of electrodes (5) being in direct contact with the electrically conductive linear bodies (31), and the first base material (1) or the second base material (2) is laminated on the wiring sheet (10) via a second resin layer (6) having a lower storage modulus than the first resin layer (4).

## Description

### TECHNICAL FIELD

The present invention relates to a laminate.

### BACKGROUND ART

For instance, Patent Literature 1 discloses, as a wiring sheet usable for a planar heater, a wiring sheet including a pseudo-sheet structure including a plurality of electrically conductive linear bodies arranged with a spacing, a cured substance layer supporting the pseudo-sheet structure, and a pair of electrodes that are in direct contact with the electrically conductive linear bodies. In the wiring sheet, the cured substance layer includes a cured substance of a curable adhesive and a storage modulus at 23 degrees C of the cured substance layer is in a range from 5.0 × 10⁶ Pa to 1.0 × 10¹⁰ Pa.

### CITATION LIST

### PATENT LITERATURE(S)

Patent Literature 1: International Publication No. WO 2021/225142

### SUMMARY OF THE INVENTION

### PROBLEM(S) TO BE SOLVED BY THE INVENTION

The wiring sheet described in Patent Literature 1 makes it possible to stabilize a resistance value of the wiring. However, it has been found that in a case where the wiring sheet described in Patent Literature 1 is placed in use between two base materials having different coefficients of linear expansion, one of the base materials may be cracked.

An object of the invention is to provide a laminate capable of preventing occurrence of a crack in a base material.

### MEANS FOR SOLVING THE PROBLEM(S)

[1] A laminate including: a first base material; a second base material having a higher linear coefficient of thermal expansion than the first base material; and a wiring sheet held between the first base material and the second base material, in which
   the wiring sheet includes a wiring body including a plurality of electrically conductive linear bodies arranged with a spacing, a first resin layer directly or indirectly supporting the wiring body, and a pair of electrodes being in direct contact with the electrically conductive linear bodies, and
   the first base material or the second base material is laminated on the wiring sheet via a second resin layer having a lower storage modulus than the first resin layer.
[2] In the laminate according to [1], a storage modulus at 23 degrees C of the second resin layer is in a range from 1.0 × 10⁴ Pa to 3.0 × 10⁵ Pa.
[3] In the laminate according to [1] or [2], a storage modulus at 23 degrees C of the first resin layer is in a range from 5.0 × 10⁶ Pa to 1.0 × 10¹⁰ Pa.
[4] In the laminate according to any one of [1] to [3], a linear coefficient of thermal expansion of the first base material is in a range from 0.01 × 10⁻⁶/degrees C to 10 × 10⁻⁶/degrees C.
[5] In the laminate according to any one of [1] to [4], a linear coefficient of thermal expansion of the second base material is in a range from 50 ×10⁻⁶/degrees C to 100 ×10⁻⁶/degrees C.
[6] In the laminate according to any one of [1] to [5], the second base material and the wiring sheet are laminated with the second resin layer interposed therebetween.

According to an aspect of the invention, it is possible to provide a laminate capable of preventing occurrence of a crack in a base material.

### BRIEF DESCRIPTION OF DRAWINGS

Fig. 1 schematically illustrates a laminate according to a first exemplary embodiment of the invention.
Fig. 2 is a cross-sectional view taken along line II-II in Fig. 1.
Fig. 3 is a cross-sectional view of a laminate according to a second exemplary embodiment of the invention.

### DESCRIPTION OF EMBODIMENT(S)

### First Exemplary Embodiment

Hereinafter, an exemplary embodiment of the invention will be described with reference to the attached drawings. The invention is by no means limited to details of the exemplary embodiment. It should be noted that some parts of the drawings are enlarged or reduced in size for the convenience of description.

### Laminate

A laminate 100 according to the exemplary embodiment includes a first base material 1, a second base material 2 having a higher linear coefficient of thermal expansion than the first base material 1, and a wiring sheet 10 held between the first base material 1 and the second base material 2, as illustrated in Fig. 1 and Fig. 2.

The wiring sheet 10 includes a wiring body 3 including a plurality of electrically conductive linear bodies 31 arranged with a spacing, a first resin layer 4 directly or indirectly supporting the wiring body 3, and a pair of electrodes 5 being in direct contact with the electrically conductive linear bodies 31.

Moreover, the first base material 1 or the second base material 2 is laminated on the wiring sheet 10 via a second resin layer 6 having a lower storage modulus than the first resin layer 4. It should be noted that in Fig. 2, the second base material 2 and the wiring sheet 10 are laminated with the second resin layer 6 interposed therebetween.

Moreover, two holes are made in the second base material 2. The two holes enable electrical connection between the pair of electrodes 5 and a power source (not illustrated).

The inventors speculate that the following is a reason why the laminate 100 according to the exemplary embodiment makes it possible to prevent occurrence of a crack in the base material.

That is to say, one reason for the occurrence of a crack in the second base material 2 is a difference in linear coefficient of thermal expansion between the first base material 1 and the second base material 2. For instance, when a temperature of the laminate 100 becomes high, the second base material 2 expands more than the first base material 1. Then, since the first base material 1 and the second base material 2 are fixed by the wiring sheet 10 held therebetween, the second base material 2 is warped to be cracked. In contrast to the above, the first base material 1 or the second base material 2 is laminated on the wiring sheet 10 via the second resin layer 6 having a lower storage modulus than the first resin layer 4. The second resin layer 6 is easily deformable due to a lower storage modulus. Thus, when the temperature of the laminate 100 becomes high, the second resin layer 6 deforms, which makes it possible to reduce warp to be generated in the second base material 2. Therefore, it is possible to prevent the occurrence of a crack in the base material.

### First Base Material

The first base material 1 is able to directly or indirectly support the wiring body 3. The first base material 1 is also able to protect one surface of the wiring sheet 10.

The linear coefficient of thermal expansion of the first base material 1 is lower than the linear coefficient of thermal expansion of the second base material 2. Therefore, the exemplary embodiment makes it possible to prevent the occurrence of a crack in the second base material 2 even though the coefficients of linear expansion differ.

The linear coefficient of thermal expansion of the first base material 1 may be 0.01 × 10⁻⁶/degrees C or more, 0.1 × 10⁻⁶/degrees C or more, or 0.5 × 10⁻⁶/degrees C or more. The linear coefficient of thermal expansion of the first base material 1 is also preferably 20 × 10⁻⁶/degrees C or less, more preferably 10 × 10⁻⁶/degrees C or less, and still more preferably 5 × 10⁻⁶/degrees C or less. It should be noted that the linear coefficient of thermal expansion is measurable by a method described in Examples described below. Conditions for measuring the linear coefficient of thermal expansion are as described later.

A material of the first base material 1 is preferably resin, glass, and the like in terms of the strength and handleability of the laminate.

When the first base material 1 is in the form of a film, a thickness of the first base material 1 is not particularly limited. The thickness of the first base material 1 is preferably 10 µm or more, more preferably 15 µm or more, and still more preferably 50 µm or more. The thickness of the first base material 1 is also preferably 10 mm or less, more preferably 5 mm or less, and still more preferably 3 mm or less.

### Second Base Material

The second base material 2 is able to directly or indirectly support the wiring body 3. The second base material 2 is also able to protect one surface of the wiring sheet 10.

The linear coefficient of thermal expansion of the second base material 2 is higher than the linear coefficient of thermal expansion of the second base material 1. Therefore, the exemplary embodiment makes it possible to prevent the occurrence of a crack in the second base material 2 even though the coefficients of linear expansion differ.

The linear coefficient of thermal expansion of the second base material 2 is preferably 30 × 10⁻⁶/degrees C or more, more preferably 45 × 10⁻⁶/degrees C or more, and still more preferably 60 × 10⁻⁶/degrees C or more. The linear coefficient of thermal expansion of the second base material 2 is preferably 200 × 10⁻⁶/degrees C or less, more preferably 150 × 10⁻⁶/degrees C or less, and still more preferably 100 × 10⁻⁶/degrees C or less. It should be noted that a method of measuring the linear coefficient of thermal expansion is as described later.

A material of the second base material 2 is preferably resin or the like in terms of the handleability and manufacturing suitability of the laminate.

Examples of the resin include polyethylene, polypropylene, polybutene, polybutadiene, polymethylpentene, polyvinyl chloride, vinyl chloride copolymer, polyethylene terephthalate, polyethylene naphthalate, polybutylene terephthalate, polyurethane, ethylene-vinyl acetate copolymer, ionomer resin, ethylene-(meth)acrylic acid copolymer, polystyrene, polycarbonate, cycloolefin polymer, and polyimide.

When the second base material 2 is in the form of a film, a thickness of the second base material 2 is not particularly limited. The thickness of the second base material 2 is preferably 10 µm or more, more preferably 30 µm or more, and still more preferably 50 µm or more. The thickness of the second base material 2 is also preferably 10 mm or less, more preferably 5 mm or less, and still more preferably 3 mm or less.

### Wiring Sheet

The wiring sheet 10 includes the wiring body 3, the first resin layer 4, and the pair of electrodes 5. The wiring sheet 10 is held between the first base material 1 and the second base material 2 and both surfaces of the wiring sheet 10 are protected by the first base material 1 and the second base material 2.

### Wiring Body

The wiring body 3 has a structure in which the plurality of electrically conductive linear bodies 31 are arranged with a spacing therebetween. Moreover, the wiring body 3 has a structure in which the plurality of electrically conductive linear bodies 31 are arranged in parallel.

The electrically conductive linear bodies 31 may each be in a linear shape or a wavy shape in a plan view of the laminate 100. Examples of the wavy shape include sine wave, rectangular wave, triangular wave, and saw-tooth wave. The wiring body 3 having, for instance, such a structure can suppress breakage of the electrically conductive linear bodies 31 when the laminate 100 is stretched in an axial direction of the electrically conductive linear bodies 31.

A volume resistivity of the electrically conductive linear bodies 31 is preferably 1.0 × 10⁻⁹ Ω•m or more, more preferably 3.0 × 10⁻⁹ Ω•m or more, and still more preferably 1.0 × 10⁻⁸ Ω•m or more. The volume resistivity of the electrically conductive linear bodies 31 is also preferably 1.0 × 10⁻³ Ω•m or less, more preferably 1.0 × 10⁻⁴ Ω•m or less, and still more preferably 1.0 × 10⁻⁵ Ω•m or less. At the volume resistivity of the electrically conductive linear bodies 31 within the above range, a surface resistance of the wiring body 3 is likely to decrease.

The volume resistivity of the electrically conductive linear bodies 31 is measured as follows. Silver paste is applied to end portions of the electrically conductive linear body 31 and to portions located 40 mm from the end portions, and the resistance of the end portions and the portions located 40 mm from the end portions is measured. Then, the cross-sectional area (unit: m²) of the electrically conductive linear bodies 31 is multiplied by the above resistance value, and the obtained value is divided by the above measured length (0.04 m), thereby calculating the volume resistivity of the electrically conductive linear bodies 31.

A shape of a cross section of the electrically conductive linear bodies 31 is not particularly limited and may be a polygonal shape, a flat shape, an elliptical shape, or a circular shape. The shape of the cross section of the electrically conductive linear bodies 31 is preferably an elliptical shape or a circular shape in terms of affinity with the first resin layer 4, or the like.

When the cross section of each of the electrically conductive linear bodies 31 is in a circular shape, a diameter D of each of the electrically conductive linear bodies 31 (see Fig. 2) is preferably in a range from 3 µm to 200 µm. In order to suppress rise in sheet resistance and improve the heat generation efficiency and dielectric breakdown resistance of the laminate 100, the diameter D of each of the electrically conductive linear bodies 31 is more preferably 4 µm or more, still more preferably 5 µm or more. The diameter D of each of the electrically conductive linear bodies 31 is more preferably 150 µm or less, still more preferably 100 µm or less, still further more preferably 50 µm or less, and yet still further more preferably 20 µm or less.

When the cross section of the electrically conductive linear bodies 31 is in an elliptical shape, the major axis is preferably in a range similar to the above range of the diameter D.

The diameter D of the electrically conductive linear bodies 31 is defined as an average value obtained by observing the electrically conductive linear bodies 31 with a digital microscope, measuring the diameter of the electrically conductive linear bodies 31 at five randomly selected locations, and averaging the measured values.

A spacing L between the electrically conductive linear bodies 31 (see Fig. 2) is preferably 0.3 mm or more, more preferably 0.5 mm or more, still more preferably 0.8 mm or more, and still further more preferably 1.5 mm or more. The spacing L between the electrically conductive linear bodies 31 is preferably 50 mm or less, more preferably 30 mm or less, still more preferably 20 mm or less, and still further more preferably 5 mm or less.

With the spacing between the electrically conductive linear bodies 31 falling within the above range, the electrically conductive linear bodies are sufficiently densely arranged, which makes it possible to improve a function of the laminate 100, such as maintaining a low resistance of the wiring body 3.

For the spacing L between the electrically conductive linear bodies 31, for instance, the electrically conductive linear bodies 31 of the wiring body 3 are observed using a digital microscope and a spacing between adjacent two of the electrically conductive linear bodies 31 is measured.

It should be noted that the spacing between adjacent two of the electrically conductive linear bodies 31 refers to a length along a direction in which the electrically conductive linear bodies 31 are arranged and also a length between facing portions of the two electrically conductive linear bodies 31 (see Fig. 2). When the electrically conductive linear bodies 31 are arranged at irregular spacings, the spacing L is an average value of the spacings between all the adjacent electrically conductive linear bodies 31.

The electrically conductive linear bodies 31, a form of which is not particularly limited, may be produced by a technique such as etching, screen printing, or inkjet printing. The electrically conductive linear bodies 31 are suitably linear bodies each including a metal wire (hereinafter, also referred to as "metal wire linear bodies"). The metal wire has high thermal conductivity, high electrical conductivity, and high handleability. The metal wire linear bodies can have significantly reduced resistance, so that an electric current necessary for the laminate 100 to generate heat can flow therethrough even when the diameter of the metal wire linear bodies is extremely reduced. This makes it possible to make the electrically conductive linear bodies 31 less visible. That is to say, using the metal wire linear bodies as the electrically conductive linear bodies 31 reduces a resistance value of the wiring body 3 and facilitates an improvement in light transmissivity. Rapid heat generation is readily achieved in the laminate 100. Further, linear bodies with a small diameter are easy to obtain as described above.

It should be noted that examples of the electrically conductive linear bodies 31 include, in addition to the metal wire linear bodies, linear bodies each including a carbon nanotube and linear bodies each including a yarn provided with electrically conductive coating.

The metal wire linear bodies may each be a linear body including a single metal wire, or may be a linear body including a plurality of metal wires twisted together.

Examples of the metal wire include wires containing metals such as copper, aluminum, tungsten, iron, molybdenum, nickel, titanium, silver, and gold, or alloys containing two or more of metals (e.g., steels such as stainless steel and carbon steel, brass, phosphor bronze, zirconium copper alloy, beryllium copper, iron-nickel, Nichrome, nickel-titanium, Kanthal, Hastelloy, and rhenium-tungsten). Moreover, the metal wire may be plated with gold, tin, zinc, silver, nickel, chromium, nickel-chromium alloy, solder, or the like or may be surface-coated with a later-described carbon material, polymer, or the like. In particular, a wire containing one or more metals selected from tungsten, molybdenum, and alloys containing these elements in terms of low volume resistivity.

Examples of the metal wire also include a metal wire coated with a carbon material. When the metal wire is coated with a carbon material, the metallic luster is reduced, thereby making it easy to render the presence of the metal wire inconspicuous. Moreover, coating the metal wire with the carbon material also inhibits metal corrosion.

Examples of the carbon material for coating the metal wire include: amorphous carbons such as carbon black, activated carbon, hard carbon, soft carbon, mesoporous carbon, and carbon fiber; graphite; fullerene; graphene; and carbon nanotube.

The electrically conductive linear bodies 31 may be linear bodies each including a yarn provided with electrically conductive coating. Examples of the yarn include a yarn spun from a resin such as nylon or polyester. Examples of the yarn also include yarns of metal fiber, carbon fiber, and ion-conductive polymer fiber. Examples of the electrically conductive coating include coating films of metal, electrically conductive polymer, and carbon material. The electrically conductive coating may be formed by plating, deposition method, or the like. The linear bodies including a yarn having the electrically conductive coating enable the yarn to maintain flexibility and enable the linear bodies to improve electrical conductivity. That is to say, a reduction in the resistance of the wiring body 3 is facilitated.

### First Resin Layer

The first resin layer 4 directly or indirectly supports the wiring body 3. The first resin layer 4 also enables stabilization of the resistance value of the wiring body 3. That is, the first resin layer 4 can fix the conductive linear bodies 31, stabilize the contact between the conductive linear bodies 31 and the electrode 5, and make it less likely for an increase in resistance value to occur.

From the point of view of stabilization of the resistance value of the wiring body 3, a storage modulus at 23 degrees C of the first resin layer 4 is preferably in a range from 5.0 × 10⁶ Pa to 1.0 × 10¹⁰ Pa. From the same point of view, the storage modulus at 23 degrees C of the first resin layer 4 is more preferably 5.0 × 10⁷ Pa or more, still more preferably 5.0 × 10⁸ Pa or more. The storage modulus at 23 degrees C of the first resin layer is more preferably 7.0 × 10⁹ Pa or less, still more preferably 4.0 × 10⁹ Pa or less.

Moreover, from the same point of view, a storage modulus at 105 degrees C of the first resin layer 4 is preferably 5.0 × 10⁷ Pa or more, more preferably 5.0 × 10⁸ Pa or more. The storage modulus at 105 degrees C of the first resin layer 4 is preferably 7.0 × 10⁹ Pa or less, more preferably 4.0 × 10⁹ Pa or less.

It should be noted that the storage modulus is measurable by a method described in Examples described later.

A thickness of the first resin layer 4 is not particularly limited. The thickness of the first resin layer 4 may be equal to or more than the diameter D of the electrically conductive linear bodies 31 or may be less than the diameter D of the electrically conductive linear bodies 31. When the thickness of the first resin layer 4 is equal to or more than the diameter D of the conductive linear bodies 31, the first resin layer 4 can contain the wiring bodies 3. When the thickness of the first resin layer 4 is less than the diameter D of the conductive linear bodies 31, the wiring body 3 is exposed from the first resin layer 4. Moreover, when the wiring body 3 is exposed from the first resin layer 4, the wiring body 3 may be exposed on a side facing the first base material 1 or exposed on a side facing the second base material 2. The thickness of the first resin layer 4 is preferably 1 µm or more, more preferably 5 µm or more, and still more preferably 10 µm or more. The thickness of the first resin layer 4 is preferably 100 µm or less, more preferably 50 µm or less, and still more preferably 30 µm or less.

From the viewpoint of setting the storage modulus within the above range, it is preferable that the first resin layer 4 is a layer formed of a cured product of a curable adhesive.

Examples of the curable adhesive include a thermosetting adhesive that cures by heat and an energy-ray-curable adhesive. Examples of the energy ray include ultraviolet rays, visible rays, infrared rays, and electron beams. It should be noted that the term "energy-ray curing" also encompasses thermal curing by heating with energy rays.

It is preferable that the curable adhesive include a thermosetting resin. The thermosetting resin is not particularly limited and specific examples thereof include an epoxy resin, a phenolic resin, a melamine resin, a urea resin, a polyester resin, a urethane resin, an acrylic resin, a benzoxazine resin, a phenoxy resin, an amine compound, and an acid anhydride compound. One of the above substances may be used alone or two or more of the above may be used in combination. Among the above, in terms of suitability for curing using an imidazole curing catalyst, an epoxy resin, a phenolic resin, a melamine resin, a urea resin, an amine compound, and an acid anhydride compound are preferably usable. In particular, in terms of exhibiting excellent curing properties, an epoxy resin, a phenolic resin, a mixture thereof, or a mixture of an epoxy resin and at least one selected from the group consisting of a phenolic resin, a melamine resin, a urea resin, an amine compound, and an acid anhydride compound is preferably usable, and an epoxy resin is preferably usable.

The epoxy resin is preferably a cyclic epoxy resin such as an aromatic epoxy resin or an alicyclic epoxy resin in terms of increasing the storage modulus of the first resin layer 4. An epoxy resin with a flexible segment such as an oxyalkylene chain tends to lower the storage modulus of the first resin layer 4.

It is preferable that the energy-ray-curable adhesive contain an energy-ray-curable resin. Examples of the energy-ray-curable resin include a compound having at least one polymerizable double bond in a molecule, and an acrylate compound having a (meth)acryloyl group is preferable.

Examples of the acrylate compound include: chain-aliphatic-skeleton-containing (meth)acrylate such as dicyclopentadiene acrylate, trimethylolpropane tri(meth)acrylate, tetramethylolmethane tetra(meth)acrylate, pentaerythritol tri(meth)acrylate, pentaerythritol tetra(meth)acrylate, dipentaerythritol monohydroxy penta(meth)acrylate, dipentaerythritol hexa(meth)acrylate, 1,4-butylene glycol di(meth)acrylate, and 1,6-hexanediol di(meth)acrylate; cyclic-aliphatic-skeleton-containing (meth)acrylate such as dicyclopentanyl di(meth)acrylate; polyalkylene glycol (meth)acrylate such as polyethylene glycol di(meth)acrylate; and oligoester (meth)acrylate, urethane (meth)acrylate oligomer, epoxy-modified (meth)acrylate, polyether (meth)acrylate excluding polyalkylene glycol (meth)acrylate, and itaconic acid oligomer.

The weight average molecular weight (Mw) of the energy-ray-curable resin is preferably 100 or more, more preferably 300 or more. The weight average molecular weight is also preferably 30,000 or less, more preferably 10,000 or less. It should be noted that the weight-average molecular weight as referred to herein is a value in terms of standard polystyrene, as measured by gel permeation chromatography (GPC).

The adhesive may contain one energy-ray-curable resin or two or more energy-ray-curable resins. For the two or more energy-ray-curable resins, a combination and ratio thereof may be selected as desired.

When the energy-ray-curable resin or the thermosetting resin is used, a photopolymerization initiator, a thermal polymerization initiator, and the like are preferably used. By using a photopolymerization initiator and a thermal polymerization initiator and the like, the polymerization reaction of the curable resin can be easily initiated, and the curing reaction can be readily controlled.

Examples of the photopolymerization initiator include photo-radical polymerization initiators such as benzophenone, acetophenone, benzoin, benzoin methyl ether, 2,4-diethylthioxanthone, 1-hydroxycyclohexyl phenyl ketone, benzyl diphenyl sulfide, tetramethylthiuram monosulfide, azobisisobutyronitrile, 2-chloroanthraquinone, diphenyl(2,4,6-trimethylbenzoyl)phosphine oxide, and bis(2,4,6-trimethylbenzoyl)-phenyl-phosphine oxide.

The examples of the photopolymerization initiator also include a photo-cationic polymerization initiator in addition to the photo-radical polymerization initiator. A photo-cationic polymerization initiator is a compound which, upon irradiation with an energy beam, generates a cationic species to initiate the curing reaction of a cationically curable compound, and which includes a cationic moiety that absorbs the energy ray and an anionic moiety that serves as a source of acid.

Examples of the photo-cationic polymerization initiator include a sulfonium salt compound, a iodonium salt compound, a phosphonium salt compound, an ammonium salt compound, an antimony acid salt compound, a diazonium salt compound, a selenium salt compound, an oxonium salt compound, and a bromine salt compound. Among the above, in terms of an excellent compatibility and an excellent preservation stability of the resulting adhesive, a sulfonium salt compound is preferable and an aromatic sulfonium salt compound having an aromatic group is more preferable.

Examples of the sulfonium salt compound include triphenylsulfonium hexafluorophosphate, triphenylsulfonium hexafluoroantimonate, and triphenylsulfonium tetrakis(pentafluorophenyl)borate.

Examples of the iodonium salt compound include diphenyliodonium tetrakis(pentafluorophenyl)borate, diphenyliodonium hexafluorophosphate, and (tricumyl)iodonium tetrakis(pentafluorophenyl)borate.

Examples of the phosphonium salt compound include tri-n-butyl(2,5-dihydroxyphenyl)phosphonium bromide and hexadecyltributylphosphonium chloride.

Examples of the ammonium salt compound include benzyltrimethylammonium chloride, phenyltributylammonium chloride, and benzyltrimethylammonium bromide.

Examples of the antimony acid salt compound include triphenylsulfonium hexafluoroantimonate, p-(phenylthio)phenyl diphenylsulfonium hexafluoroantimonate, and diallyliodonium hexafluoroantimonate.

Examples of the thermal polymerization initiator include thermal radical polymerization initiators such as: hydrogen peroxides; peroxodisulfates such as ammonium peroxodisulfate, sodium peroxodisulfate, and potassium peroxodisulfate; azo compounds such as 2,2'-azobis(2-amidinopropane) dihydrochloride, 4,4'-azobis(4-cyanovaleric acid), 2,2'-azobisisobutyronitrile, and 2,2'-azobis(4-methoxy-2,4-dimethylvaleronitrile); and organic peroxides such as benzoyl peroxide, lauroyl peroxide, peracetic acid, persuccinic acid, di-t-butyl peroxide, t-butyl hydroperoxide, and cumene hydroperoxide.

The examples of the thermal polymerization initiators also include a thermal cationic polymerization initiator in addition to the above thermal radical polymerization initiator. The thermal cationic polymerization initiator is a compound capable of generating a cationic species that initiates polymerization upon heating. Examples of the thermal cationic polymerization initiator include a sulfonium salt, a quaternary ammonium salt, a phosphonium salt, a diazonium salt, and a iodonium salt. Among these, sulfonium salts are preferred from the viewpoint of easy availability and the likelihood of obtaining products excellent in adhesion and transparency.

Examples of the sulfonium salt include triphenylsulfonium tetrafluoroborate, triphenylsulfonium hexafluoroantimonate, and triphenylsulfonium hexafluoroarsenate.

Examples of the quaternary ammonium salt include tetrabutylammonium tetrafluoroborate, tetrabutylammonium hexafluorophosphate, and tetrabutylammonium hydrogensulfate.

Examples of the phosphonium salt include ethyltriphenylphosphonium hexafluoroantimonate, and tetrabutylphosphonium hexafluoroantimonate.

Examples of the diazonium salt include benzenediazonium chloride. Examples of the iodonium salt include diphenyliodonium hexafluoroarsenate, bis(4-chlorophenyl)iodonium hexafluoroarsenate, and phenyl(4-methoxyphenyl)iodonium hexafluoroarsenate.

One of the above polymerization initiators may be used alone or two or more of the above may be used in combination.

When forming a crosslinked structure using these polymerization initiators, the amount thereof is preferably in a range from 0.1 parts by mass to 30 parts by mass per 100 parts by mass of the energy-ray curable resin or thermosetting resin, more preferably in a range from 0.5 parts by mass to 20 parts by mass, and still more preferably in a range from 1 part by mass to 10 parts by mass.

Moreover, when the thermosetting resin is used, a curing catalyst such as an imidazole curing catalyst may be used.

In the exemplary embodiment, the curable adhesive may contain a flexibility-adjusting component, together with an energy-ray curable resin or a thermosetting resin, in order to facilitate maintenance of the sheet shape prior to curing. Examples of a polymer usable as the flexibility-adjusting component include a phenoxy resin, a polyolefin resin or a modified form thereof, a polyamideimide resin, a polyimide resin, a rubber resin, and an acrylic resin.

One of the above flexibility-adjusting components may be used alone or two or more of the above may be used in combination.

When the curable adhesive used in the exemplary embodiment contains a flexibility-adjusting component, the total amount of the energy-ray curable resin and the thermosetting resin contained in the adhesive is preferably in a range from 15 parts by mass to 300 parts by mass, more preferably in a range from 30 parts by mass to 250 parts by mass, and still more preferably in a range from 60 parts by mass to 200 parts by mass, relative to 100 parts by mass of the flexibility-adjusting component, from the viewpoint of adjusting the storage modulus of the first resin layer 4 within the above-mentioned range. Moreover, when the adhesive contains the energy-ray-curable resin or the thermosetting resin but no flexibility adjusting component, the storage modulus of the first resin layer 4 tends to become excessively high.

In the exemplary embodiment, it is preferable that the curable adhesive contain no filler. When the adhesive contains no filler, it is possible to prevent the storage modulus at 23 degrees C of the first resin layer 4 from becoming excessively high.

Incidentally, the curable adhesive may contain a filler, insofar as the storage modulus of the first resin layer 4 at 23 degrees C can be adjusted within the above-mentioned range.

Examples of the filler include: inorganic powders such as silica, alumina, talc, calcium carbonate, titanium white, red iron oxide, silicon carbide, and boron nitride; spherical beads obtained by spheronizing inorganic powders; single-crystal fibers; and glass fibers. Among the above, a silica filler and an alumina filler are preferable. One of the fillers may be used alone or two or more of the above may be used in combination.

The curable adhesive may contain another component. Examples of the other component include known additives such as organic solvents, coupling agents, flame retardants, tackifiers, ultraviolet absorbers, antioxidants, preservatives, antifungal agents, plasticizers, defoaming agents, and wettability modifiers.

### Electrodes

The electrodes 5 are used to supply current to the electrically conductive linear bodies 31. The electrodes 5 form a pair. The electrodes 5 are in direct contact with the electrically conductive linear bodies 31. Then, the electrodes 5 are arranged to be electrically connected to opposite ends of the electrically conductive linear bodies 31.

The electrode 5 can be formed using known electrode materials. Examples of the electrode material include an electrically conductive paste such as silver paste, a metal foil such as copper foil, and a metal wire. When the electrode material is a metal wire, it may include a single metal wire but preferably includes two or more metal wires.

When the electrode material is a metal foil or a metal wire, examples of the metal foil or the metal wire include metals such as copper, aluminum, tungsten, iron, molybdenum, nickel, titanium, silver, and gold or alloys containing two or more metals, such as steels such as stainless steel and carbon steel, brass, phosphor bronze, zirconium copper alloy, beryllium copper, iron nickel, Nichrome, nickel titanium, Kanthal, Hastelloy, and rhenium tungsten. Moreover, the metal foil or the metal wire may be plated with gold, tin, zinc, silver, nickel, chromium, nickel-chromium alloy, solder, or the like.

A width of at least one of the electrodes 5 is preferably 10 mm or less in a plan view of the laminate 100, more preferably 3 mm or less. The width of the electrode is also preferably 0.1 mm or more, more preferably 0.5 mm or more. It should be noted that, when at least one of the electrodes is a metal wire, the width of the electrode is the diameter of the metal wire, and when two or more metal wires are used, the width of one electrode refers to the sum of the diameters of the respective metal wires.

A thickness of the electrodes 5 is preferably 2 µm or more, more preferably 5 µm or more, and still more preferably 10 µm or more. The thickness of the electrodes 5 is preferably 200 µm or less, more preferably 100 µm or less, still more preferably 50 µm or less, and still further more preferably 25 µm or less. As long as the thickness of the electrode 5 is within the above-mentioned range, high electrical conductivity and low resistance can be achieved, thereby keeping the resistance value with the pseudo-sheet structure low. Moreover, a sufficient strength as an electrode is obtainable. It should be noted that the electrodes are each provided by the metal wire, the thickness of the electrode refers to the diameter of the metal wire.

### Second Resin Layer

The second resin layer 6 is provided between the first base material 1 or the second base material 2 and the wiring sheet 10. The second resin layer 6 has a lower storage modulus than the first resin layer 4. The second resin layer 6 makes it possible to prevent the occurrence of a crack in the second base material 2. In the exemplary embodiment, the second base material 2 and the wiring sheet 10 are laminated with the second resin layer 6 interposed therebetween.

From the point of view of preventing a crack, a storage modulus at 23 degrees C of the second resin layer 6 is preferably in a range from 1.0 × 10⁴ Pa to 3.0 × 10⁵ Pa. From the same point of view, the storage modulus at 23 degrees C of the second resin layer 6 is more preferably 4.0 × 10⁴ Pa or more, still more preferably 8.0 × 10⁴ Pa or more. The storage modulus at 23 degrees C of the second resin layer 6 is more preferably 2.5 × 10⁵ Pa or less, still more preferably 2.0 × 10⁵ Pa or less.

Moreover, from the same point of view, a storage modulus at 105 degrees C of the second resin layer 6 is preferably 5.0 × 10³ Pa or more, more preferably 5.0 × 10⁴ Pa or more. The storage modulus at 105 degrees C of the second resin layer 6 is preferably 4.0 × 10⁴ Pa or less, more preferably 3.0 × 10⁴ Pa or less.

It should be noted that the storage modulus is measurable by a method described in Examples described later.

A thickness of the second resin layer 6 is not particularly limited. The thickness of the second resin layer 6 is preferably 1 µm or more, more preferably 5 µm or more, and still more preferably 10 µm or more. The thickness of the second resin layer 6 is preferably 1,000 µm or less, more preferably 500 µm or less, and still more preferably 300 µm or less.

From the viewpoint of exhibiting excellent performance as a pressure-sensitive adhesive layer and from the viewpoint of setting the storage modulus within the above-mentioned range, the second resin layer 6 is preferably the following pressure-sensitive adhesive layer.

The pressure-sensitive adhesive layer can be formed of a pressure-sensitive adhesive obtained by crosslinking (heat crosslinking) a pressure-sensitive adhesive composition (hereinafter sometimes referred to as "pressure-sensitive adhesive composition P") containing, for example, a (meth)acrylic acid ester polymer (A) and a crosslinking agent (B), or an energy-ray-curable component (C), or both thereof. Incidentally, it is preferable that the pressure-sensitive adhesive composition P preferably further contains a photopolymerization initiator (D) as desired. Moreover, (meth)acrylic acid herein means both an acrylic acid and a methacrylic acid. The same applies to other similar terms. The term "polymer" herein shall be understood to also encompass "copolymer," unless otherwise specified.

When the pressure-sensitive adhesive composition contains the energy-ray-curable component (C), the pressure-sensitive adhesive layer obtained by crosslinking the pressure-sensitive adhesive composition, at the stage of the pressure-sensitive adhesive sheet, that is, prior to being applied to an adherend, has not yet been cured by an energy ray and exhibits a relatively low storage modulus. Thus, the stress generated upon lamination to an adherend can be mitigated. As a result, even when the pressure-sensitive adhesive layer is laminated to a surface of an adherend having irregularities, the pressure-sensitive adhesive layer readily follows the irregularities, whereby the occurrence of gaps, lifting, or the like in the vicinity of the irregularities is suppressed, and excellent lamination property to the adherend is exhibited.

It is preferable that the (meth)acrylic acid ester polymer (A) contains, as monomer units constituting the polymer, an alkyl (meth)acrylate and a monomer having a reactive functional group in a molecule (a reactive-functional-group-containing monomer).

The (meth)acrylic acid ester polymer (A) can exhibit desirable pressure-sensitive adhesion by containing, as monomer units constituting the polymer, an alkyl (meth)acrylate. As the alkyl (meth)acrylate, an alkyl (meth)acrylate having an alkyl group with 1 to 20 carbon atoms is preferable. The alkyl group may be linear or branched and may have a cyclic structure.

Examples of the alkyl (meth)acrylates having an alkyl group with 1 to 20 carbon atoms include (meth)acrylic acid methyl, (meth)acrylic acid ethyl, (meth)acrylic acid propyl, (meth)acrylic acid n-butyl, (meth)acrylic acid n-pentyl, (meth)acrylic acid n-hexyl, (meth)acrylic acid 2-ethylhexyl, (meth)acrylic acid isooctyl, (meth)acrylic acid n-decyl, (meth)acrylic acid n-dodecyl, (meth)acrylic acid myristyl, (meth)acrylic acid palmityl, (meth)acrylic acid stearyl, (meth)acrylic acid cyclohexyl, (meth)acrylic acid isobornyl, and (meth)acrylic acid adamantyl. One of the above may be used alone, or two or more thereof may be used in combination.

Among the above, an alkyl (meth)acrylate having an alkyl group having 4 to 20 carbon atoms is preferable as the alkyl (meth)acrylate. As the alkyl (meth)acrylates having an alkyl group having 4 to 20 carbon atoms, (meth)acrylic acid n-butyl, (meth)acrylic acid 2-ethylhexyl, (meth)acrylic acid isooctyl, (meth)acrylic acid isobornyl and the like are preferable. From the viewpoint of achieving excellent pressure-sensitive adhesion, (meth)acrylic acid n-butyl, (meth)acrylic acid 2-ethylhexyl, and (meth)acrylic acid isobornyl are more preferable, and acrylic acid n-butyl, acrylic acid 2-ethylhexyl, acrylic acid isobornyl and the like are particularly preferable.

The (meth)acrylic acid ester polymer (A) preferably contains 40 mass% or more of an alkyl (meth)acrylate as monomer units constituting the polymer, more preferably 50 mass% or more, still more preferably 60 mass% or more, and particularly preferably 70 mass% or more. When the (meth)acrylic acid ester polymer (A) contains 40 mass% or more of an alkyl (meth)acrylate, the polymer can exhibit favorable pressure-sensitive adhesion. Further, the (meth)acrylic acid ester polymer (A) preferably contains 99 mass% or less of an alkyl (meth)acrylate as monomer units constituting the polymer, more preferably 95 mass% or less, and still more preferably 90 mass% or less. When the content of the alkyl (meth)acrylate is 99 mass% or less, another monomer component can be suitably introduced into the (meth)acrylic acid ester polymer (A). In particular, when the (meth)acrylic acid ester polymer (A) contains a hydroxyl group-containing monomer as a monomer constituting the polymer, the (meth)acrylic acid ester polymer (A) preferably contains 87 mass% or less of an alkyl (meth)acrylate as monomer units constituting the polymer, and more preferably 83 mass% or less.

The (meth)acrylic acid ester polymer (A) contains a reactive functional group-containing monomer as monomer units constituting the polymer, whereby the polymer reacts with the crosslinking agent (B) described later through the reactive functional group derived from the reactive functional group-containing monomer, thereby forming a crosslinked structure (three-dimensional network structure), and consequently a pressure-sensitive adhesive having the desired cohesive force is obtained.

As the reactive functional group-containing monomers contained as monomer units in the (meth)acrylic acid ester polymer (A), preferred examples include monomers having a hydroxyl group in a molecule (hydroxyl group-containing monomers), monomers having a carboxyl group in a molecule (carboxyl group-containing monomers), and monomers having an amino group in a molecule (amino group-containing monomers). One of the reactive functional group-containing monomers may be used alone, or two or more thereof may be used in combination.

Among the reactive functional group-containing monomers, hydroxyl group-containing monomers or carboxyl group-containing monomers are preferable from the viewpoint of facilitating adjustment of the crosslinking density and easily obtaining a pressure-sensitive adhesive having the desired cohesive force. From the viewpoint of pressure-sensitive adhesion and resistance to moisture-heat whitening, hydroxyl group-containing monomers are preferable.

Examples of the hydroxyl group-containing monomers include hydroxyalkyl (meth)acrylates such as 2-hydroxyethyl (meth)acrylate, 2-hydroxypropyl (meth)acrylate, 3-hydroxypropyl (meth)acrylate, 2-hydroxybutyl (meth)acrylate, 3-hydroxybutyl (meth)acrylate, and 4-hydroxybutyl (meth)acrylate. Among these, hydroxyalkyl (meth)acrylates having a hydroxyalkyl group having 1 to 4 carbon atoms are preferable. Specifically, preferred examples include 2-hydroxyethyl (meth)acrylate and 4-hydroxybutyl (meth)acrylate, and particularly 2-hydroxyethyl acrylate and 4-hydroxybutyl acrylate are preferable. One of the above may be used alone, or two or more thereof may be used in combination.

Examples of the carboxyl group-containing monomers include ethylenically unsaturated carboxylic acids such as acrylic acid, methacrylic acid, crotonic acid, maleic acid, itaconic acid, and citraconic acid. Among these, acrylic acid is preferable from the viewpoint of the cohesive force of the resulting (meth)acrylic acid ester polymer (A). One of the above may be used alone, or two or more thereof may be used in combination.

The (meth)acrylic acid ester polymer (A) preferably contains 1 mass% or more of the reactive functional group-containing monomer as monomer units constituting the polymer, more preferably 3 mass% or more, and still more preferably 5 mass% or more. When the reactive functional group-containing monomer is a hydroxyl group-containing monomer, the (meth)acrylic acid ester polymer (A) preferably contains 5 mass% or more thereof, more preferably 8 mass% or more, and still more preferably 10 mass% or more. Further, when the reactive functional group-containing monomer is a hydroxyl group-containing monomer, the content is preferably less than 25 mass%, more preferably 20 mass% or less, and still more preferably 16 mass% or less. Further, the (meth)acrylic acid ester polymer (A) preferably contains 50 mass% or less of the reactive functional group-containing monomer as monomer units constituting the polymer, more preferably 40 mass% or less, and still more preferably 30 mass% or less.

It is also preferable that the (meth)acrylic acid ester polymer (A) contains, as monomer units constituting the polymer, a nitrogen-atom-containing monomer. By incorporating a nitrogen atom-containing monomer as a constitutional unit into the polymer, a predetermined polarity can be imparted to the pressure-sensitive adhesive, thereby allowing the pressure-sensitive adhesive to exhibit excellent affinity even for an adherend having a certain degree of polarity, such as glass. Examples of the nitrogen atom-containing monomer include, in addition to the aforementioned amino group-containing monomer as the reactive functional group-containing monomer, a monomer having an amide group and a monomer having a nitrogen-containing heterocycle. Among the above, a monomer having a nitrogen-containing heterocycle is preferable in terms of imparting an appropriate rigidity to the (meth)acrylic acid ester polymer (A).

Examples of the nitrogen atom-containing monomer that may also be used include N-vinylcarboxylic acid amide, (meth)acrylamide, N-methyl(meth)acrylamide, N-methylol(meth)acrylamide, N-tert-butyl(meth)acrylamide, N,N-dimethyl(meth)acrylamide, N,N-ethyl(meth)acrylamide, N,N-dimethylaminopropyl(meth)acrylamide, N-isopropyl(meth)acrylamide, N-phenyl(meth)acrylamide, dimethylaminopropyl(meth)acrylamide, and N-vinylcaprolactam.

One of the nitrogen atom-containing monomer may be used alone, or two or more thereof may be used in combination.

Examples of the monomer having a nitrogen-containing heterocycle include N-(meth)acryloylmorpholine, N-vinyl-2-pyrrolidone, N-(meth)acryloylpyrrolidone, N-(meth)acryloylpiperidine, N-(meth)acryloylpyrrolidine, N-(meth)acryloylaziridine, aziridinylethyl (meth)acrylate, 2-vinylpyridine, 4-vinylpyridine, 2-vinylpyrazine, 1-vinylimidazole, N-vinylcarbazole, and N-vinylphthalimide. Among these, N-(meth)acryloylmorpholine is preferable because of exhibiting superior pressure-sensitive adhesion, and particularly N-acryloylmorpholine (4-acryloylmorpholine) is preferable.

When the (meth)acrylic acid ester polymer (A) contains, as monomer units constituting the polymer, a monomer having a nitrogen-containing heterocycle, the polymer preferably contains 0.5 mass% or more of a nitrogen atom-containing monomer, more preferably 1 mass% or more, and still more preferably 3 mass% or more. Further, the (meth)acrylic acid ester polymer (A) preferably contains 20 mass% or less of a monomer having a nitrogen-containing heterocycle as monomer units constituting the polymer, more preferably 15 mass% or less, and still more preferably 8 mass% or less. When the content of the monomer having a nitrogen-containing heterocycle is within the above range, the resulting pressure-sensitive adhesive can effectively exhibit excellent adhesion to adherends such as glass.

The (meth)acrylic acid ester polymer (A) may optionally contain other monomers as monomer units constituting the polymer. Examples of the other monomers include (meth)acrylic acid alkoxyalkyl esters such as (meth)acrylic acid methoxyethyl and (meth)acrylic acid ethoxyethyl, vinyl acetate, and styrene. One of the above may be used alone, or two or more thereof may be used in combination.

The (meth)acrylic acid ester polymer (A) is preferably a linear polymer. By being a linear polymer, entanglement of molecular chains is more likely to occur, which can be expected to improve cohesive force, thereby providing an improved pressure-sensitive adhesive.

The polymerization mode of the (meth)acrylic acid ester polymer (A) may be a random copolymer or may be a block copolymer.

The weight average molecular weight of the (meth)acrylic acid ester polymer (A) is preferably 200,000 or more, more preferably 300,000 or more, and still more preferably 400,000 or more. When the lower limit of the weight average molecular weight of the (meth)acrylic acid ester polymer (A) is at least the above value, the second resin layer and the laminate exhibit excellent long-term durability.

Further, the weight average molecular weight of the (meth)acrylic acid ester polymer (A) is preferably 2,000,000 or less, more preferably 1,500,000 or less, still more preferably 1,000,000 or less, and still further more preferably 800,000 or less. When the upper limit of the weight average molecular weight of the (meth)acrylic acid ester polymer (A) is at most the above value, at least one of the lamination property or the adhesion of the resulting pressure-sensitive adhesive to an adherend is improved.

In the pressure-sensitive adhesive composition P, one of the (meth)acrylic acid ester polymer (A) may be used alone or two or more thereof may be used in combination.

The crosslinking agent (B) can crosslink the (meth)acrylic acid ester polymer (A) by heating the pressure-sensitive adhesive composition P, thereby enabling favorable formation of a three-dimensional network structure. As a result, the cohesive force of the resulting pressure-sensitive adhesive is further improved.

As the crosslinking agent (B), any compound that can react with the reactive functional group of the (meth)acrylic acid ester polymer (A) may be used. Examples of the crosslinking agent (B) include an isocyanate crosslinking agent, epoxy crosslinking agent, amine crosslinking agent, melamine crosslinking agent, aziridine crosslinking agent, hydrazine crosslinking agent, aldehyde crosslinking agent, oxazoline crosslinking agent, metal alkoxide crosslinking agent, metal chelate crosslinking agent, metal salt crosslinking agent, and ammonium salt crosslinking agent. Among these, when the reactive functional group of the (meth)acrylic acid ester polymer (A) is a hydroxyl group, it is preferable to use an isocyanate crosslinking agent having excellent reactivity with the hydroxyl group. When the reactive functional group of the (meth)acrylic acid ester polymer (A) is a carboxyl group, it is preferable to use an epoxy crosslinking agent having excellent reactivity with the carboxyl group. One of the crosslinking agent (B) may be used alone or two or more thereof may be used in combination.

The isocyanate crosslinking agent contains at least a polyisocyanate compound. Examples of the polyisocyanate compounds include aromatic polyisocyanates such as tolylene diisocyanate, diphenylmethane diisocyanate, and xylylene diisocyanate; aliphatic polyisocyanates such as hexamethylene diisocyanate; and alicyclic polyisocyanates such as isophorone diisocyanate and hydrogenated diphenylmethane diisocyanate. Further, the examples include biuret derivatives and isocyanurate derivatives thereof, as well as adducts which are reaction products with low molecular active hydrogen-containing compounds such as ethylene glycol, propylene glycol, neopentyl glycol, trimethylolpropane, and castor oil. Among these, from the viewpoint of reactivity with hydroxyl groups, trimethylolpropane-modified aromatic polyisocyanates are preferable, and in particular, it is preferable to use at least one of trimethylolpropane-modified tolylene diisocyanate or trimethylolpropane-modified xylylene diisocyanate.

Examples of the epoxy crosslinking agent include 1,3-bis(N,N-diglycidylaminomethyl)cyclohexane, N,N,N',N'-tetraglycidyl-m-xylylenediamine, ethylene glycol diglycidyl ether, 1,6-hexanediol diglycidyl ether, trimethylolpropane diglycidyl ether, diglycidylaniline, and diglycidylamine. Among these, from the viewpoint of reactivity with carboxyl groups, 1,3-bis(N,N-diglycidylaminomethyl)cyclohexane is preferable.

The content of the crosslinking agent (B) in the pressure-sensitive adhesive composition P is preferably 0.01 parts by mass or more, more preferably 0.05 parts by mass or more, and still more preferably 0.1 parts by mass or more, relative to 100 parts by mass of the (meth)acrylic acid ester polymer (A). Further, the content thereof is preferably 3 parts by mass or less, more preferably 2 parts by mass or less, and still more preferably 1 part by mass or less. When the content of the crosslinking agent (B) is within the above range, the degree of crosslinking becomes appropriate, and the resulting pressure-sensitive adhesive can be more easily adjusted to a favorable value of storage modulus as described above, thereby being improved.

By containing the energy-ray-curable component (C), the pressure-sensitive adhesive composition P, when crosslinked (thermally crosslinked), provides a pressure-sensitive adhesive that is energy-ray curable. It is presumed that, by curing upon irradiation with energy rays after being applied to an adherend, the energy-ray-curable component (C) polymerizes with each other, and the polymerized energy-ray-curable component (C) entangles with the crosslinked structure (three-dimensional network structure) of the (meth)acrylic acid ester polymer (A). The pressure-sensitive adhesive having such a higher-order structure exhibits high cohesive force and shows high coating film strength.

The energy-ray-curable component (C) is not particularly limited as long as it is a component that cures upon irradiation with energy rays to provide the above effects, and may be a monomer, an oligomer, or a polymer, or a mixture thereof. Among these, multifunctional acrylate monomers having excellent compatibility with the (meth)acrylic acid ester polymer (A) and the like can be preferably mentioned.

Examples of the multifunctional acrylate monomers include difunctional types such as tricyclodecanedimethanol di(meth)acrylate, 1,4-butanediol di(meth)acrylate, 1,6-hexanediol di(meth)acrylate, neopentyl glycol di(meth)acrylate, polyethylene glycol di(meth)acrylate, neopentyl glycol adipate di(meth)acrylate, hydroxypivalic acid neopentyl glycol di(meth)acrylate, dicyclopentenyl di(meth)acrylate, caprolactone-modified dicyclopentenyl di(meth)acrylate, ethylene oxide-modified phosphoric acid di(meth)acrylate, di(acryloxyethyl)isocyanurate, allyl cyclohexyl di(meth)acrylate, ethoxylated bisphenol A diacrylate, and 9,9-bis[4-(2-acryloyloxyethoxy)phenyl]fluorene; trifunctional types such as trimethylolpropane tri(meth)acrylate, dipentaerythritol tri(meth)acrylate, propionic acid-modified dipentaerythritol tri(meth)acrylate, pentaerythritol tri(meth)acrylate, propylene oxide-modified trimethylolpropane tri(meth)acrylate, tris(acryloxyethyl)isocyanurate, and ε-caprolactone-modified tris(2-(meth)acryloxyethyl)isocyanurate; tetrafunctional types such as diglycerin tetra(meth)acrylate and pentaerythritol tetra(meth)acrylate; pentafunctional types such as propionic acid-modified dipentaerythritol penta(meth)acrylate; and hexafunctional types such as dipentaerythritol hexa(meth)acrylate and caprolactone-modified dipentaerythritol hexa(meth)acrylate. Among the above, it is preferable to use at least one of ε-caprolactone-modified tris(2-(meth)acryloxyethyl)isocyanurate or tricyclodecanedimethanol di(meth)acrylate. One of the above may be used alone, or two or more thereof may be used in combination. Further, from the viewpoint of compatibility with the (meth)acrylic acid ester polymer (A), the multifunctional acrylate monomer preferably has a molecular weight of less than 1000.

From the viewpoint of facilitating adjustment of the resulting pressure-sensitive adhesive to a desired value of storage modulus as described above, the content of the energy-ray-curable component (C) in the pressure-sensitive adhesive composition P is preferably 1 part by mass or more, more preferably 2 parts by mass or more, still more preferably 3 parts by mass or more, and still further more preferably 5 parts by mass or more, relative to 100 parts by mass of the (meth)acrylic acid ester polymer (A). On the other hand, from the viewpoint of preventing the energy-ray-curable component (C) from phase-separating from the (meth)acrylic acid ester polymer (A) and from the viewpoint of facilitating adjustment of the above-described storage modulus to a desired value, the content of the energy-ray-curable component (C) is preferably 50 parts by mass or less, more preferably 30 parts by mass or less, still more preferably 20 parts by mass or less, and still further more preferably 7.5 parts by mass or less, relative to 100 parts by mass of the (meth)acrylic acid ester polymer (A).

When ultraviolet rays are used as the energy rays for curing the energy-ray-curable pressure-sensitive adhesive, the pressure-sensitive adhesive composition P preferably further contains a photopolymerization initiator (D). By containing such a photopolymerization initiator (D), the energy-ray-curable component (C) can be efficiently polymerized, and the polymerization curing time and the irradiation dose of the energy rays can be reduced.

Examples of the photopolymerization initiator (D) include benzophenone, acetophenone, benzoin, benzoin methyl ether, benzoin ethyl ether, benzoin isopropyl ether, benzoin isobutyl ether, benzoin benzoate, benzoin methyl benzoate, benzoin dimethyl ketal, 2,4-diethylthioxanthone, 1-hydroxycyclohexyl phenyl ketone, benzyl diphenyl sulfide, tetramethylthiuram monosulfide, azobisisobutyronitrile, benzyl, dibenzyl, diacetyl, β-chloroanthraquinone, 4-(2-hydroxyethoxy)phenyl(2-hydroxy-2-propyl)ketone, 2-benzothiazole-N,N-diethyldithiocarbamate, 2,4,6-trimethylbenzoyl diphenylphosphine oxide, and bis(2,4,6-trimethylbenzoyl)phenylphosphine oxide. One of the above may be used alone, or two or more thereof may be used in combination.

The content of the photopolymerization initiator (D) in the pressure-sensitive adhesive composition P is preferably 0.1 parts by mass or more, more preferably 1.0 part by mass or more, and still more preferably 5.0 parts by mass or more, relative to 100 parts by mass of the energy-ray-curable component (C). Further, the content thereof is preferably 35 parts by mass or less, more preferably 25 parts by mass or less, and still more preferably 15 part by mass or less. When the content of the photopolymerization initiator (D) is within this range, it undergoes cleavage without problems upon irradiation with energy rays, and the curability of the energy-ray-curable component (C) is further improved. Further, the above-described storage modulus is more easily satisfied.

If desired, various additives that are commonly used in acrylic pressure-sensitive adhesives may be used in the pressure-sensitive adhesive composition P. Examples of the various additives include silane coupling agents, antistatic agents, tackifiers, antioxidants, light stabilizers, plasticizers, fillers, and refractive index modifiers.

### Production Method of Laminate

A method for producing the laminate 100 ilm is not particularly limited. The laminate 100 can be produced, for example, by the following steps.

First, a step of producing a wiring body film provided with a wiring body 3 is carried out. In this step, a thermosetting adhesive for forming the first resin layer 4 is applied onto a release film to form a coating film. Next, the coating film is dried to produce an adhesive layer. Next, the conductive linear body 31 is placed on the adhesive layer while being arranged, thereby forming the wiring body 3. For example, in a state where an adhesive layer with a release film is disposed on the outer peripheral surface of a drum member, the drum member is rotated while winding the conductive linear body 31 spirally around the adhesive layer. Thereafter, the bundle of the conductive linear body 31 wound spirally is cut along the axial direction of the drum member. Thus, the wiring body 3 is formed and disposed on the adhesive layer. In this manner, a wiring body film in which the wiring body 3 is formed on the adhesive layer with a release film is obtained. According to this method, for example, by rotating the drum member while moving the feeding portion of the conductive linear body 31 along a direction parallel to the axis of the drum member, it is easy to adjust the spacings L between the adjacent conductive linear bodies 31 in the wiring body 3.

Next, a step of providing a pair of electrodes 5 on the first base material 1 is carried out. In this step, a pair of electrodes 5 can be provided on the first base material 1, for example, by printing a conductive paste or the like in a predetermined arrangement and then drying it.

Next, a step of placing the wiring body film on the first base material 1 provided with the pair of electrodes 5 and curing the thermosetting adhesive is carried out. In this step, the wiring body film is laminated onto the first base material 1 provided with the pair of electrodes 5 so that the pair of electrodes 5 come into contact with both end portions of the conductive linear bodies 31 in the wiring body 3 of the wiring body film. Then, after peeling off the release film, the thermosetting adhesive is subjected to a predetermined heat treatment to form the first resin layer 4, thereby forming a wiring sheet 10 on the first base material 1.

On the other hand, a step of producing a protective film provided with the second base material 2 and the second resin layer 6 is carried out. In this step, the pressure-sensitive adhesive composition P for forming the second resin layer 6 is applied onto the second base material 2 to form a coating film, thereby producing the protective film. It is preferable, as illustrated in Figs. 1 and 2, to provide two holes in the second base material 2.

Next, a step of placing the protective film on the first base material 1 provided with the wiring sheet 10 and crosslinking the pressure-sensitive adhesive composition P is carried out. In this step, the protective film is laminated onto the first base material 1 provided with the wiring sheet 10 such that, in a plan view, the two holes of the protective film overlap with the pair of electrodes 5, and the coating film of the pressure-sensitive adhesive composition P of the protective film comes into contact with the wiring sheet 10. Then, by subjecting the coating film of the pressure-sensitive adhesive composition P to predetermined energy-ray irradiation, the second resin layer 6 is formed, thereby producing the laminate 100.

### Advantage(s) of First Exemplary Embodiment

According to the first exemplary embodiment, the following advantages can be achieved.
(1) According to the first exemplary embodiment, the second resin layer 6 is easily deformable due to a lower storage modulus. Thus, when the temperature of the laminate 100 becomes high, the second resin layer 6 deforms, which makes it possible to reduce warp to be generated in the second base material 2. Thus, it is possible to prevent the occurrence of a crack in the second base material 2.
(2) According to the first exemplary embodiment, by setting the storage modulus of the second resin layer 6 at 23 degrees C to 1.0×10⁴ Pa or more and 3.0×10⁶ Pa or less, the second resin layer 6 can be made easily deformable, and warp generated in the second base material 2 can be alleviated.
(3) According to the first exemplary embodiment, by means of the first resin layer 4, the conductive linear bodies 31 can be fixed, deformation in the thickness direction inside the laminate 100 can be suppressed, contact between the conductive linear bodies 31 and the electrodes 5 can be stabilized, and the resistance value of the wiring body 3 can be stabilized.
(4) According to the first exemplary embodiment, by setting the storage modulus of the first resin layer 4 at 23 degrees C to 5.0×10⁶ Pa or more and 1.0×10¹⁰ Pa or less, the conductive linear bodies 31 can be fixed while preventing breakage of the connection portion between the conductive linear bodies 31 and the electrodes 5 when deformation is applied to the laminate 100.
(5) The laminate 100 according to the exemplary embodiment can be produced by the above-described method for producing the laminate in a relatively simple manner.

### Second Exemplary Embodiment

Next, a second exemplary embodiment of the invention will be described with reference to the attached drawings. The invention is by no means limited to details of the exemplary embodiment. It should be noted that some parts of the drawings are enlarged or reduced in size for the convenience of description.

The second exemplary embodiment is different from the first exemplary embodiment in that the first base material 1 and the wiring sheet 10 are laminated with the second resin layer 6 interposed therebetween, as illustrated in a cross-sectional view of a laminate 100A.

In the following description, portions mainly relating to differences from the first exemplary embodiment will be described, and redundant explanations will be omitted or simplified. The same components as those in the first exemplary embodiment are denoted by the same reference signs to simplify or omit an explanation of the components.

The laminate 100A according to the exemplary embodiment includes the first base material 1, the second base material 2 having a higher linear coefficient of thermal expansion than the first base material 1, and the wiring sheet 10 held between the first base material 1 and the second base material 2, as illustrated in Fig. 3. The wiring sheet 10 includes a wiring body 3 including a plurality of electrically conductive linear bodies 31 arranged with a spacing, the first resin layer 4 directly or indirectly supporting the wiring body 3, and a pair of electrodes 5 being in direct contact with the electrically conductive linear bodies 31. Moreover, the first base material 1 and the wiring sheet 10 are laminated with the second resin layer 6 having a lower storage modulus than the first resin layer 4.

### Advantage(s) of Second Exemplary Embodiment

According to the second exemplary embodiment, the advantages (1) to (4) described in the first exemplary embodiment can be achieved.

### Modification of Embodiments

The invention is not limited to the above exemplary embodiments and includes any modification, improvement, and the like as long as the object of the invention can be achieved.

For example, in the above exemplary embodiments, the laminate 100 includes the film-shaped first base material 1, but is not limited thereto. For example, the first base material 1 may be a base material formed into a three-dimensional shape. In such a case, the wiring sheet 10 can be attached to the first base material 1, which is the adherend, by means of the first resin layer 4 or the second resin layer 6.

In the above-described second exemplary embodiment, the cross-sectional view of the laminate 100A is modified in that the first base material 1 and the wiring sheet 10 are laminated with the second resin layer 6 interposed therebetween; however, the modification is not limited thereto. For example, two other modifications can be given. One modification is an example in which, in the first exemplary embodiment, the wiring sheet 10 is turned upside down such that the electrode 5 is provided on the side of the second base material 2. The other modification is an example in which, in the second exemplary embodiment, the wiring sheet 10 is turned upside down such that the electrode 5 is provided on the side of the second base material 2.

### Examples

The invention will be described below in more detail with reference to Examples. The invention is by no means limited to these Examples.

Further, laminates obtained in Examples were evaluated as follows.

### Crack Evaluation

After the laminate was left to stand at 105 degrees C for 1000 hours, the presence or absence of cracks in the base material layer of each laminate was examined using a digital microscope.

### Measurement of Storage Modulus

A cylindrical test sample having a diameter of 8 mm and a thickness of 1 mm was prepared from the same composition as that used to form the layer to be measured. The storage modulus of the test sample was measured using a dynamic viscoelasticity measuring apparatus (MCR300, manufactured by Anton Paar) under the following conditions: a parallel plate with a diameter of 8 mm as the measuring fixture, a test starting temperature of -20 degrees C, a test ending temperature of 150 degrees C, a heating rate of 3 degrees C/min, a shear strain of 0.05%, and a frequency of 1 Hz.

### Measurement of Linear Coefficient of Thermal Expansion

A base material was cut into a rectangular shape of 4.5 mm × 20 mm to prepare a test sample. A linear coefficient of thermal expansion of the test sample was measured using a thermomechanical analyzer (TMA4000SE, manufactured by Netzsch Japan) under the following conditions: tensile load of 2 g, temperature range from 23 degrees C to 105 degrees C, and heating rate of 5 degrees C/min.

### Preparation Example 1

A curable adhesive was obtained by blending 100 parts by mass of a phenoxy resin (YX7200B35, manufactured by Mitsubishi Chemical Corporation) with 170 parts by mass of a multifunctional hydrogenated bisphenol A diglycidyl ether epoxy compound (YX8000, manufactured by Mitsubishi Chemical Corporation), 0.2 parts by mass of a silane coupling agent (KBM-4803, manufactured by Shin-Etsu Chemical Co., Ltd.), 2 parts by mass of a thermal cationic polymerization initiator (SANEID SI-B3, manufactured by Sanshin Chemical Industry Co., Ltd.), and 2 parts by mass of a thermal cationic polymerization initiator (SANEID SI-B7, manufactured by Sanshin Chemical Industry Co., Ltd.).

### Preparation Example 2

### Preparation of (meth)acrylic acid ester polymer (A)

A (meth)acrylic acid ester polymer (A) was prepared by copolymerizing 65 parts by mass of 2-ethylhexyl acrylate, 5 parts by mass of 4-acryloylmorpholine, 15 parts by mass of isobornyl acrylate, and 15 parts by mass of 2-hydroxyethyl acrylate. The molecular weight of the (meth)acrylic acid ester polymer (A) was measured, and the weight-average molecular weight (Mw) was 500,000. Furthermore, the glass transition temperature (Tg, in degrees C) of the (meth)acrylic acid ester polymer (A) was calculated to be -36.5 degrees C according to the Fox equation, based on the glass transition temperatures (Tg) of the respective monomers constituting the (meth)acrylic acid ester polymer (A) as homopolymers.

### Preparation of Pressure-sensitive Adhesive Composition

A coating solution of a pressure-sensitive adhesive composition was obtained by mixing 100 parts by mass (in terms of solid content; the same shall apply hereinafter) of the obtained (meth)acrylic acid ester polymer (A), 0.18 parts by mass of a crosslinking agent (B), namely trimethylolpropane-modified tolylene diisocyanate, 7 parts by mass of an energy-ray curable component (C), namely ε-caprolactone-modified tris-(2-acryloyloxyethyl) isocyanurate, 0.7 parts by mass of a mixture of a photopolymerization initiator (D), namely benzophenone and 1-hydroxycyclohexyl phenyl ketone in a 1:1 mass ratio, and 0.28 parts by mass of a silane coupling agent, namely 3-glycidoxypropyltrimethoxysilane, followed by sufficient stirring and dilution with methyl ethyl ketone.

### Preparation Example 3

### Preparation of Pressure-sensitive Adhesive Composition

A coating solution of a pressure-sensitive adhesive composition was obtained by mixing 100 parts by mass of the (meth)acrylic acid ester polymer (A) obtained in Preparation Example 2, 0.15 parts by mass of a crosslinking agent (B), namely trimethylolpropane-modified tolylene diisocyanate, 5 parts by mass of an energy-ray curable component (C), namely ε-caprolactone-modified tris-(2-acryloyloxyethyl) isocyanurate, 0.5 parts by mass of a photopolymerization initiator (D), namely 2,4,6-trimethylbenzoyl-diphenylphosphine oxide, and 0.25 parts by mass of a silane coupling agent, namely 3-glycidoxypropyltrimethoxysilane, followed by sufficient stirring and dilution with methyl ethyl ketone.

### Preparation Example 4

### Preparation of (meth)acrylic acid ester polymer (A)

A (meth)acrylic acid ester polymer (A) was prepared by copolymerizing 30 parts by mass of 2-ethylhexyl acrylate, 25 parts by mass of n-butyl acrylate, 5 parts by mass of 4-acryloylmorpholine, 15 parts by mass of isobornyl acrylate, and 25 parts by mass of 2-hydroxyethyl acrylate. The molecular weight of the (meth)acrylic acid ester polymer (A) was measured, and the weight-average molecular weight (Mw) was 600,000.

### Preparation of Pressure-sensitive Adhesive Composition

A coating solution of a pressure-sensitive adhesive composition was obtained by mixing 100 parts by mass of the obtained (meth)acrylic acid ester polymer (A), 0.2 parts by mass of a crosslinking agent (B), namely trimethylolpropane-modified tolylene diisocyanate, 8.0 parts by mass of an energy-ray curable component (C), namely ε-caprolactone-modified tris-(2-acryloyloxyethyl) isocyanurate, 0.8 parts by mass of a photopolymerization initiator (D), namely 2,4,6-trimethylbenzoyl-diphenylphosphine oxide, and 0.2 parts by mass of a silane coupling agent, namely 3-glycidoxypropyltrimethoxysilane, followed by sufficient stirring and dilution with methyl ethyl ketone.

### Example 1

### Preparation of Wiring Body Film

An adhesive sheet was prepared by coating a curable adhesive obtained in Preparation Example 1 onto a release film having a thickness of 38 µm (SP-382150, manufactured by Lintec Corporation) so as to have a thickness of 15 µm, and cutting the coated product into a rectangle of 250 mm × 320 mm. As a conductive linear body, a gold-plated tungsten wire having a diameter of 10 µm was prepared (hereinafter also referred to simply as "wire"). Next, the obtained adhesive sheet was wound around a drum member having a rubber outer peripheral surface in such a manner that the surface of the pressure-sensitive adhesive layer faced outward and no wrinkles were formed, and both ends of the adhesive sheet in the circumferential direction were fixed with a double-sided tape. The wire wound on a bobbin was first attached to the surface of the pressure-sensitive adhesive layer of the adhesive sheet located near an end portion of the drum member. Then, while unwinding the wire from the bobbin, the wire was wound onto the drum member, and the drum member was gradually moved in a direction parallel to the drum axis so that the wire was helically wound around the drum member at equal intervals of 3 mm. As a result, a wiring body was formed in such a manner that 96 wires were arranged on the surface of the adhesive. Thereafter, the wire was cut, and the wiring body was removed from the drum member. The wiring body was then cut into a width of 40×82 mm so as to obtain 12 wires, thereby preparing a wiring body film.

### Preparation of Substrate with Electrodes

A strip-shaped electrode having a thickness of 17 µm was formed by screenprinting silver paste with a width of 2 mm and an inter-electrode distance of 7.8 mm onto a glass substrate serving as a first base material and having a thickness of 2 mm and a linear coefficient of thermal expansion of 3.3 × 10⁻⁶/degrees C, followed by drying at 150 degrees C for 30 minutes. Thereafter, electroless plating was applied to the strip-shaped electrode to fabricate a substrate with electrodes.

### Formation of Wiring Sheet

The obtained wiring body film was laminated onto the obtained substrate with electrodes such that the electrodes were positioned at both ends of the wires. Thereafter, heating was performed at 120 degrees C and 0.5 MPa for 30 minutes to cure the adhesive, thereby forming a first resin layer and forming a wiring sheet on the first base material.

The storage modulus of the first resin layer was 2.2 × 10⁹ Pa at 23 degrees C and 1.6 × 10⁹ Pa at 105 degrees C.

### Preparation of Protective Sheet

On a cycloolefin polymer film having a thickness of 100 µm (production name: ZF16, manufactured by Zeon Corporation) serving as a second base material, a coating solution of the pressure-sensitive adhesive composition obtained in Preparation Example 2 was applied so as to have a thickness of 100 µm, and then cut into a rectangle of 50 mm × 120 mm. Thereafter, two circular holes each having a diameter of 5 mm were punched out such that the distance between the centers of the two circular holes was 7.8 mm, thereby preparing a protective sheet.

Table 1 shows the linear coefficient of thermal expansion of the second base material.

### Preparation of Laminate

A protective sheet was laminated onto the first base material provided with a wiring sheet such that the electrodes of the wiring sheet were aligned with the circular holes of the protective sheet. Thereafter, ultraviolet light having a wavelength of 365 nm was irradiated under conditions of an irradiance of 200 mW/cm² and an exposure dose of 1000 mJ/cm² to form a second resin layer, thereby obtaining a laminate.

Cracks of the obtained laminate were evaluated. Table 1 also shows storage moduli at 23 degrees C and 105 degrees C of the second resin layer.

### Example 2

A laminate was prepared in the same manner as in Example 1 except that the cycloolefin polymer film (product name: 'ZF16', manufactured by Zeon Corporation) used as the protective sheet was replaced with a polycarbonate film (product name: 'L-100', manufactured by Teijin Limited).

### Example 3

A laminate was prepared in the same manner as in Example 1 except that the coating solution of the pressure-sensitive adhesive composition obtained in Preparation Example 2 was replaced with the coating solution of the pressure-sensitive adhesive composition obtained in Preparation Example 3.

### Comparative 1

A laminate was prepared in the same manner as in Example 1 except that the coating solution of the pressure-sensitive adhesive composition obtained in Preparation Example 2 was replaced with the coating solution of the pressure-sensitive adhesive composition obtained in Preparation Example 4.

### Comparative 2

A laminate was prepared in the same manner as in Example 1, except that the coating solution of the pressure-sensitive adhesive composition obtained in Preparation Example 2 was replaced with the coating solution of the pressure-sensitive adhesive composition obtained in Preparation Example 4, and the cycloolefin polymer film (product name: 'ZF16', manufactured by Zeon Corporation) used as the protective sheet was replaced with a polycarbonate film (product name: 'L-100', manufactured by Teijin Limited).

**Table 1**

| | Linear Coefficient of Thermal Expansion of Second Base Material (×10⁻⁶/°C) | Storage Modulus at 23°C of Second Resin Layer (MPa) | Storage Modulus at 105°C of Second Resin Layer (MPa) | Result of Crack Evaluation |
|---|---|---|---|---|
| Ex. 1 | 63 | 0.14 | 0.021 | Not Cracked |
| Ex. 2 | 88 | 0.14 | 0.021 | Not Cracked |
| Ex. 3 | 63 | 0.16 | 0.024 | Not Cracked |
| Comp. 1 | 63 | 0.38 | 0.045 | Cracked |
| Comp. 2 | 88 | 0.38 | 0.045 | Cracked |

As shown in Table 1, the laminates obtained in Examples 1 to 3 showed favorable results in the evaluation of cracks. Accordingly, it was confirmed that, according to the invention, a laminate capable of preventing the occurrence of cracks in the base material can be obtained.

### EXPLANATION OF CODES

1...first base material, 2...second base material, 3...wiring body, 31...electrically conductive linear body, 4...first resin layer, 5...electrode, 6...second resin layer, 10...wiring sheet, 100, 100A...laminate.

## Claims

1. A laminate comprising:
a first base material;
a second base material having a higher linear coefficient of thermal expansion than the first base material; and
a wiring sheet held between the first base material and the second base material, wherein
the wiring sheet comprises a wiring body including a plurality of electrically conductive linear bodies arranged with a spacing, a first resin layer directly or indirectly supporting the wiring body, and a pair of electrodes being in direct contact with the electrically conductive linear bodies, and
the first base material or the second base material is laminated on the wiring sheet via a second resin layer having a lower storage modulus than the first resin layer.

2. The laminate according to claim 1, wherein a storage modulus at 23 degrees C of the second resin layer is in a range from 1.0 × 10⁴ Pa to 3.0 × 10⁵ Pa.

3. The laminate according to claim 1 or 2, wherein a storage modulus at 23 degrees C of the first resin layer is in a range from 5.0 × 10⁶ Pa to 1.0 × 10¹⁰ Pa.

4. The laminate according to claim 1 or 2, wherein a linear coefficient of thermal expansion of the first base material is in a range from 0.01 × 10⁻⁶/degrees C to 10 × 10⁻⁶/degrees C.

5. The laminate according to claim 1 or 2, wherein a linear coefficient of thermal expansion of the second base material is in a range from 50 × 10⁻⁶/degrees C to 100 × 10⁻⁶/degrees C.

6. The laminate according to claim 1 or 2, wherein the second base material and the wiring sheet are laminated with the second resin layer interposed therebetween.
